

Aug. 26, 1947.

L. MARICK

2,426,315

STATIC FREE BRUSH

Filed Sept. 25, 1943

Fig. 1



Fig. 2



Fig. 3

INVENTOR.  
LOUIS MARICK

BY  
Lester J. Bullock  
ATTORNEY

## UNITED STATES PATENT OFFICE

2,426,315

## STATIC FREE BRUSH

Louis Marick, Grosse Pointe Farms, Mich., assignee to United States Rubber Company, New York, N. Y., a corporation of New Jersey

Application September 25, 1943, Serial No. 503,756

3 Claims. (Cl. 15—159)

1

This invention relates to brushes the bristles of which will not accumulate static electric charges.

Hand, floor and other brushes are commonly provided with hair or fibrous bristles which are non-conductors when dry, and when one of these brushes is moved over a non-conducting surface a static charge may be produced upon the bristles and a static spark result. If a brush of this type is so used in places where inflammable materials are located, the brush may produce static sparks that will cause a fire.

Brushes provided with hair or other bristles which generate static electricity are used in munition factories to brush up small quantities of powder and when a static spark results it may cause a serious fire. A similar fire hazard is caused by the use of such brushes in various places where volatile gases are present.

The present invention contemplates brushes which will dissipate static electric charges or fail to produce such charges and as a result will not produce static sparks.

Static free brushes such as herein contemplated are well adapted for use in munition factories to brush up dry powder, in rooms where volatile gases are present, for brushing clothes or hair or for other uses where static electric charges would be objectionable.

A static free brush is produced in accordance with the present invention by depositing upon the bristles thereof a thin electric conducting coating such, for example, as a coating of conductive rubber or conductive resinous material, and by making the head in which the bristles are mounted and brush handle conductive so that a conductive path will be provided from the bristles to the head and handle to permit a static charge at the bristles to reach the hand of the person using the brush and disperse over his body.

The various features of the present invention will be further understood from the following description when read in connection with the accompanying drawing illustrating several brushes having the static free construction of the present invention.

In the drawing:

Fig. 1 is a perspective view of a paint brush of usual construction except for the static free feature of the present invention;

Fig. 2 is a perspective view of a similar type of brush having an electric conducting plastic head and handle;

Fig. 3 is a perspective view of a floor brush, and;

Fig. 4 is a perspective view of a clothes brush.

2

The brush shown in Fig. 1 of the drawing has a wooden handle 10, a metal ferrule or head 11 and the bristle portion 12. Such a brush, of usual construction, may be purchased on the market and have the static free features of the present invention imparted thereto by dipping the bristle portion 12 thereof in a solution of conducting rubber cement to thereby provide a conductive path along the bristles to the metal ferrule or head 11, and the handle 10 is readily made conductive by providing the same with the conductive coating 13 which obviously should contact the metal head 11 so that a conductive path will be provided along the bristles to the head 11 and from the head along the handle to the hand of the person using the brush.

It is important that the bristles 12 be treated with a thin solution of conductive cement so that the conductive coating provided upon the bristles will not appreciably increase the size or stiffness of the individual bristles. Good results have been secured by dipping the bristles in a conductive rubber cement of the following formula:

|    |                 |      |
|----|-----------------|------|
| 25 | Rubber          | 100  |
|    | Zinc oxide      | 15   |
|    | Antioxidant     | 0.35 |
|    | Accelerator     | 2.00 |
|    | Stearic acid    | 7.00 |
| 30 | Sulphur         | 0.75 |
|    | Acetylene black | 85   |

Such a cement is preferably thinned with gasoline to a watery consistency. For example, good results have been obtained by employing a solution of 769 grams of gasoline containing 120 grams of cement. The bristles of the brush are dipped into the solution and the excess of the solution is "thrown" off the brush. One dip will usually suffice to give proper conductive properties to the bristles. However, for practical purposes it is desirable to give the brush about four dippings. Such a coating on the bristles is extremely thin and is not readily perceptible to the eye or to the touch, but is sufficiently conductive to disperse static charges.

The mass of bristles 12 may be formed of various types of hair or of synthetic fibers or filaments such as rayon, nylon or other plastics, all of which may be treated by dipping them into the solution of conductive cement of the above example. The bristles 12 instead of being treated with conductive rubber such as above described may be treated with synthetic rubber, plastic or resin containing conductive carbon.

55 The wooden handle 10 may be coated with a

rubber composition such as given in the above example. However, for coating the handle portion of the brush it is deemed preferable to employ the conductive properties of acetylene black used as a varnish, lacquer or other synthetic resin coating. An example of such coating is as follows:

|                      | Per cent |
|----------------------|----------|
| Resins               | 12.9     |
| Tung oil             | 23.2     |
| Other vegetable oils | 8.2      |
| Acetylene black      | 23.2     |
| Mineral spirits      | 32.5     |

This coating may be applied to the brush handle by painting, spraying, or dipping and in the case of the brush shown in Fig. 1, it is important that the coating upon both the bristles and the handle be so applied that the coating shall reach or over-lap the metal ferrule of the brush so as to form a continuous conducting path from the bristles to the brush handle.

In the construction shown in Fig. 2 the bristles 12 may be the same as the bristles 12 of Fig. 1 and may be rendered conductive by the treatment above described. These bristles, however, are shown as mounted in a plastic head 14 having formed integrally therewith the handle 15. The plastic material of which such head and handle are formed may be molded to the shape shown with the upper ends of the bristles 12 embedded in the head 14. The head and handle may be formed of an electric conducting composition formed of hard rubber, phenol formaldehyde, methyl methacrylate, vinyl chloride acetate, polyvinyl alcohol and the like. A sufficient amount of acetylene black is added to such compound to render it conductive so that a static charge created by the bristles 12 may travel along the head and handle to the hand of the person using the brush to dissipate such charge.

In Fig. 3 of the drawing there is shown a floor brush of the usual construction comprising the bristles 16, the head 17 in which the bristles are mounted and handle 18 and both the head and handle may be formed of wood as usual. The bristles 16 may be rendered conductive by treating them the same as the bristles 12 above described. The head 17 is preferably provided with a conductive coating 19 similar to the coating 13 above described and which should be so applied that it will form a conductive path from the upper ends of the bristles 16 to the handle 18, which handle is preferably given a conducting coating 20 similar to the coating 13 above described. When the floor brush of Fig. 3 is so treated a conductive path will be provided upwardly along the bristles 16 to the head 17 and along the handle 18 to the hands of the person using the floor brush.

In Fig. 4 of the drawing there is shown a clothes brush having the bristles 21 mounted in the head

22 which may be formed of wood or plastic material as heretofore. The bristles 21 are preferably treated similar to the bristles 12 to make them electrically conductive and the head 22 is preferably provided with a conducting coating 23 which should be so applied that it will cover the top and side portions of the head 22 and contact the bristles 21 so that any static charge produced by the bristles may travel along these bristles to the head 22 and from the latter to the hand of the person using the brush.

The brushes above described have an electrical resistance varying from about 30,000 ohms to 200,000 ohms depending mainly upon the force exerted on the brush while brushing. This resistance value is sufficient to cause the dissipation of any static that might be accumulated by the brush.

Having thus described my invention, what I claim and desire to protect by Letters Patent is:

1. A brush which when used in a dry condition will remain static free, comprising a head having bristles secured therein and a handle extending from the head, the handle and head being coated with a conductive material to disperse static charges, and the bristles having a thin electrically conducting coating disposed thereupon so as not to bond the contacting bristles together, to thereby provide a conducting path from the bristles to the handle.

2. A brush which when used in a dry condition will remain static free, comprising a head having bristles secured therein and a handle extending from the head, the handle and head having a conductive outer surface adapted to disperse static charges, and the bristles having a thin electrically conducting coating disposed thereupon so as not to bond the contacting bristles together, to thereby provide a conducting path from the bristles to the handle.

3. A brush which when used in a dry condition will remain static free, comprising a rigid non-metallic head having non-metallic bristles secured therein, the head having a conductive outer surface adapted to disperse static charges, and the bristles having a thin electrically conducting coating of plastic material disposed thereupon so as not to bond the contracting bristles together, to thereby provide a conductive path from the bristles over the outer surface of the head.

LOUIS MARICK.

#### REFERENCES CITED

The following references are of record in the file of this patent:

#### UNITED STATES PATENTS

| Number    | Name           | Date          |
|-----------|----------------|---------------|
| 2,304,210 | Scott et al.   | Dec. 8, 1942  |
| 1,725,852 | Cressler       | Aug. 27, 1929 |
| 2,302,003 | Cadwell et al. | Nov. 17, 1942 |